

## UNITED STATES PATENT OFFICE.

FREDERICK M. BECKET, OF NEW YORK, N. Y., ASSIGNOR TO ELECTRO METALLURGICAL COMPANY, A CORPORATION OF WEST VIRGINIA.

## PROCESS OF MAKING MOLYBDENUM STEEL.

No Drawing.

Application filed November 19, 1925. Serial No. 70,188.

This invention relates to the manufacture of molybdenum steels, and comprises a process whereby molybdenum in the form of sulfid is availed of for this purpose, without resorting to preliminary roasting or other conversion. The molybdenum sulfid is conveniently used in the form of the native mineral molybdenite ( $MoS_2$ ) or concentrates containing the same, although the invention 10 contemplates the employment of molybdenum sulfid from other sources when available.

It is well-known that molybdenum steel may be made by any one of several so-called 15 "direct" processes, i. e. by processes which do not involve the preparation of metallic molybdenum or of a molybdenum alloy. In the practice of these direct processes it has hitherto been customary to introduce molybdenum into the steel furnace or crucible as an oxide of molybdenum or as a molybdate. When derived from molybdenite ore or concentrate, preparation of the oxide or of the molybdate has hitherto involved a roasting 20 operation whereby the molybdenum content of the ore was converted into molybdenum oxide or, under certain conditions when the roasting charge contained lime or iron oxide, into calcium molybdate and iron molybdate, 25 respectively. Even when any of the aforesaid chemical compounds of molybdenum have been prepared from the ore in the wet way by leaching and precipitation methods, 30 oxidation or preliminary roasting of the molybdenite or a charge mixture containing it has been characteristic of the process as 35 a whole.

According to the present invention molybdenum sulfid is brought as such into reactive 40 relation to the steel bath. My investigations have shown that under suitable conditions of practice the molybdenum content of the sulfid is recovered completely or in amount 45 sufficiently high to represent an entirely practicable recovery ratio; and what is of vital importance from the commercial aspect, this recovery is effected with little or no attendant increase in the sulphur content of the finished metal. In other words, in the 50 practice of the present invention the unit cost of the molybdenum contained in the

finished steel may in good practice be made to approach very closely, and practically to equal, that of the molybdenum content of the original ore or concentrate. 55

The following specific examples illustrate preferred procedures, as carried out in the basic electric furnace:

I. Molybdenite concentrate analyzing 54.15% molybdenum and corresponding approximately to 90%  $MoS_2$  was added to a heat of steel in a basic-lined electric furnace in such amount that the molybdenum in the concentrate added was 0.43% of the weight of the steel in the furnace. The addition 60 was made in this case after the first or oxidizing slag had been removed but prior to the attainment of those strongly reducing conditions which are characterized by a slag of the "carbide" type. This was followed by 65 furnace additions of washed metal, high-carbon ferromanganese and low-carbon ferrochrome, in the order stated. Three hours after the addition of molybdenite concentrate to the bath, and thirty minutes after 70 the addition of low-carbon ferrochrome, the heat was poured and treated in the ladle with ferrosilicon. The finished steel had the following composition: 75

|    | Per cent. | 80 |
|----|-----------|----|
| C  | 0.37      |    |
| Si | 0.35      |    |
| Mn | 0.81      |    |
| P  | 0.011     |    |
| S  | 0.012     | 85 |
| Cr | 1.12      |    |
| Mo | 0.44      |    |

The molybdenum contained in the molybdenite concentrate was recovered completely 90 in the tapped metal, within the usual limits of accuracy of sampling and analysis.

II. Molybdenite concentrate of the composition above-mentioned was added to a heat of steel in a basic-lined electric furnace 95 during the final reducing period thirty minutes before pouring. It was preceded by additions of washed metal and low-carbon ferro-chrome and was followed by a furnace addition of high-carbon ferro-manganese. 100 The amount of molybdenum thus added as molybdenite was equivalent to 0.40% of the

metal charge. The steel, which was treated in the ladle with ferrosilicon, had the following composition:

|       | Per cent. |
|-------|-----------|
| 5 C   | 0.40      |
| Si    | 0.27      |
| Mn    | 0.68      |
| P     | 0.012     |
| S     | 0.017     |
| 10 Cr | 1.12      |
| Mo    | 0.35      |

Of the molybdenum contained in the  $\text{MoS}_2$ , 88% was recovered in the tapped metal.

The invention is of course not restricted to the basic electric furnace process of making steel; it can also be used in the open-hearth and acid electric furnace processes.

20 Molybdenite and its concentrate are ordinarily procured in granular or powder form. If a sintered or agglomerated product is desired, suitable fluxing and agglomerating agents may be added, such as boric

25 oxid, glass, fluorspar, silica and basic compounds, including compounds of the alkali metals, without departure from the present invention, provided that the process of incorporating said fluxes and agglomerants

30 preserves the chemical identity of the molybdenum sulfid, or provided that said process brings about only in part the chemical conversion of the sulfid into other product or products.

35 It will be understood by those skilled in

the art that the temperature and composition of the steel and of the slag, as well as the time allowed for their reaction with molybdenum sulfid, may exert a marked effect upon the percentage recovery of molybdenum in the finished steel, and also upon the sulphur content of the latter. More especially in the case of open-hearth practice it is preferable under certain conditions to add the molybdenite in successive batches rather 45 early in the progress of the heat, and to distribute it over the surface of the bath, rather than to make the entire addition at one time and at one location within the furnace.

I claim:

1. Process of making molybdenum steel, comprising bringing molybdenum sulfid into reactive relation with a steel bath in the absence of abnormal reducing conditions.

2. Process of making molybdenum steel, comprising bringing molybdenite into reactive relation with a steel bath in the absence of abnormal reducing conditions.

3. Process of making molybdenum steel, comprising bringing a molybdenite concentrate into reactive relation with a steel bath in the absence of abnormal reducing conditions.

4. Process of making molybdenum steel, comprising agglomerating molybdenum sulfid and bringing the agglomerate into reactive relation with a steel bath in the absence of abnormal reducing conditions.

In testimony whereof, I affix my signature.

FREDERICK M. BECKET.